

Nov. 13, 1962

H. W. COATES ET AL

3,063,454

NON-WOVEN PRODUCTS

Filed Feb. 26, 1959



1

3,063,454

## NON-WOVEN PRODUCTS

Herbert W. Coates and Roland A. Frate, Charlotte, N.C., assignors to Celanese Corporation of America, New York, N.Y., a corporation of Delaware  
Filed Feb. 26, 1959, Ser. No. 795,857  
23 Claims. (Cl. 128--290)

The present invention relates to reinforcement of non-woven fibrous structures such as sanitary napkins and to other non-woven fibrous structures.

Non-woven webs are especially suited for applications where softness and porosity are called for, such materials being relatively inexpensive to manufacture. Because of the absence of interlocking as in knitting or weaving, however, non-woven unbonded webs are characterized by extremely low strengths.

It is an object of the present invention to provide a reinforced non-woven structure of considerably increased strength.

It is a further object to provide a reinforced, strong non-woven structure having the reinforcement firmly embedded in the structure.

Another object of the invention is to provide procedures for producing novel reinforced, strong non-woven structures.

Still another object is to provide non-woven coverings for disposable items such as sanitary napkins or the like.

Other objects and advantages of the invention will become apparent from the following detailed description and claims.

In accordance with one aspect of the invention, a fibrous structure is formed of potentially adhesive fibers and of other fibers containing an activating agent such as a solvent, plasticizer or swelling agent for the potentially adhesive fibers. The activating agent, advantageously upon application of pressure and/or heat, attacks the potentially adhesive fibers and causes them to be bonded to the other fibers. Such bonding of the other fibers into the matrix is ensured by virtue of the fact that the only source for activating agent for the potentially adhesive fibers in the other fibers.

In accordance with another aspect of the invention the potentially adhesive fibers are included in a non-woven web and the other fibers are included in yarns arranged to serve as a reinforcement for the web. If sufficient heat and/or pressure are employed, and if the yarns contain sufficient activating agent, the activating agent may be caused to migrate sufficiently from the yarns to effect bonding of the fibers in the web to one another in addition to bonding of the potentially adhesive fibers in the web to the reinforcing yarns. If desired, prior to application of heat and pressure a second non-woven web may be superposed on the reinforcing yarns containing activating agent to form a non-woven product having an embedded reinforcement. Any number of layers of non-woven webs and yarn reinforcements may be alternated.

The patterns in which the reinforcement yarns are laid down will determine the ultimate strength of the article. Approximately equal strengths in longitudinal and transverse directions of the non-woven can be attained by employing parallel yarns of the same composition spaced equally warp-wise and fill-wise. If the yarns are not of the same composition and/or the spacing between parallel yarns is varied, differential strengths warp-wise and fill-wise can be attained, as desired. One particularly useful grid arrangement of yarns includes a plurality of parallel yarns laid down in one direction and superposed by a plurality of additional yarns extending at 90° angles to the first-named yarns substantially in the same plane. The yarns need not be woven or otherwise interlocked, since the potentially adhesive fibers when activated will

2

bind the crossing yarns to one another as well as to the potentially adhesive fibers.

The non-woven web may be composed in whole or in part of potentially adhesive fibers representative examples of which include polyamides such as nylon, polyesters such as polyethylene terephthalate, acrylonitrile polymers and copolymers, olefin and olefinic ester polymers and copolymers such as polyethylene, polypropylene, polyvinyl chloride, poly-vinyl acetate, and the like. Especially good results are achieved with organic acid esters of cellulose such as cellulose acetate, cellulose propionate, cellulose butyrate, cellulose acetate formate, cellulose acetate propionate, cellulose acetate butyrate, and the like. Of these, cellulose acetate is preferred.

Advantageously the potentially adhesive fibers comprise more than about half of the non-woven web by weight. The component fibers may be crimped or straight and may range in denier from about 2.0 or less up to about 8.0 or even more. The non-woven web can be formed in conventional manner as by air blowing, carding, or the like, and may be partially bonded in conventional manner. Its weight and thickness will vary with the intended end use. For most purposes the weight will range from about 0.10 to 1.0 and preferably about 0.2 to 0.5 ounce per square yard.

The reinforcing yarns may comprise monofilaments, a plurality of continuous filaments, plied yarns, spun staple yarns, or the like. The yarns may comprise any of the fibrous materials hereinabove recited and they may additionally comprise cotton or rayon, preferably high tenacity rayon having a tenacity in excess of about 5.0 grams per denier such as is obtained by saponification of cellulose acetate. Yarns having tenacities in excess of 3.0 grams per denier can be used in such small amounts that they will not alter the feel of the non-woven product although they will impart appreciable reinforcement.

In any given specimen the yarns preferably comprise inert fibers of chemical composition different from that of the potentially adhesive fibers so that the activating agent with which the yarn is wet will selectively attack the potentially adhesive fibers. However, it is possible to utilize component yarns of the same chemical composition as the potentially adhesive fiber to obtain specific end use properties. Alternatively, the individual yarns can comprise a blend of inert fibers and of potentially adhesive fibers, or the reinforcement can comprise yarns of inert fibers alternated with yarns of potentially adhesive fibers.

The activating agent for the potentially adhesive fiber can comprise a volatile solvent therefor but preferably it comprises a plasticizer which may or may not be volatile. Thus, when the potentially adhesive fibers are cellulose acetate, if the reinforcing yarns are cellulose, i.e. cotton or preferably high tenacity rayon, the bonding may be effected with solvents such as acetone or methylene chloride but is better effected with high boiling organic esters of carboxylic acids such as alkyl or aryl esters of citric acid, adipic acid, maleic acid, phthalic acid, or organic esters of inorganic acids such as tributyl phosphate, tricresyl phosphate or alkoxy alkyl esters of these inorganic polybasic acids or organic polybasic acids, high-boiling ethers such as butyl ether of ethylene glycol, methyl ether of ethylene glycol, etc., high-boiling esters of polyhydric alcohols such as triacetin, glycol diacetate and diacetin. The activating agents may be diluted with water, alcohol or other poor swelling agent to decrease the activation of the potentially adhesive fibers. The activating agent is incorporated in the reinforcing yarns preferably by a coating technique, e.g. immersing, dipping, spraying, kiss rolls, or the like, followed by wiping to remove excess liquid to prevent dripping. The amount of activating

agent picked up can be varied widely and may range from about 2 to 20 and preferably 5 to 10% by weight of the yarns.

Materials produced in accordance with the invention can be used as components for building up laminates, for impregnation with plastics in making shaped structures, and the like. They are especially suited for use as covers for sanitary napkins in which application their strength, softness and relatively low cost are especially beneficial. Whereas a non-woven web in native state, or even after partial bonding and reinforcement with a wide mesh woven backing, cannot retain a safety pin or other fastener, the novel non-wovens can be held in place by pinning with no difficulty. For this end use, the non-woven web is preferably applied to both surfaces of the reinforcing yarns. The web ranges in weight from about 0.10 to 0.60 and preferably 0.20 to 0.40 ounce per square yard. The reinforcing yarns may range in denier from about 30 to 150 and are preferably laid parallel to one another, spaced about  $\frac{1}{8}$  to  $\frac{1}{4}$  inch apart. Preferably a second set of yarns, similarly constituted, is laid cross-wise directly over the first yarns. The amount of plasticizer in the yarns may range from about 2 to 20 and preferably about 5 to 10% by weight.

The accompanying drawing illustrates a preferred procedure and a representative product of the invention in the form of a sanitary napkin, this procedure and product being described in further detail in Examples I and II hereinbelow.

In the drawing,

FIGURE 1 is an exploded diagrammatic view of an assembled product of the invention before bonding;

FIGURE 2 is a view of the product assembled in FIGURE 1 after bonding; and

FIGURE 3 is a schematic elevational view of the component layers of a sanitary napkin prior to folding.

In FIG. 1, the exploded view of the laminate shows the superimposed relationship of outer webs of unbonded cellulose acetate webs 11, 12 to the longitudinal and transverse regenerated cellulose yarns 13 and 14, respectively.

In FIG. 2, the component webs 11 and 12 are not independently identifiable. Yarns 13, 14 are bonded at their crossing points as well as being bonded to the fibers of the web to form a single strong structure 15. Numerous fibers within the product 15 are bonded to one another even without directly contacting yarns 13 or 14, due to migration of the plasticizer initially contained in yarns 13, 14.

In FIG. 3 there is shown the stacked pad layers plus cover layer for forming a sanitary napkin. The layers comprise the conventional three sheets of tissue paper 16, web of viscose fiber 17, two sheets of tissue paper 18, layer of wood pulp fiber 19, sheet of water repellent tissue 20, four sheets of tissue 21, another layer of wood pulp fiber 22, another sheet of tissue 23, eight sheets of tissue 24 and a cover layer 25. In accordance with the present invention this cover layer is constituted by the reinforced non-woven web shown in FIG. 2.

The invention is more fully described in the following examples.

#### Example I

An unbonded carded-web, weighing about 0.3 ounce per square yard and composed of 3 denier cellulose acetate fibers about 2 inches long, was placed on a flat table top. High tenacity rayon yarns, made by saponifying steamed and stretched cellulose acetate multifilament yarn, comprising 40 filaments each of 0.75 denier and twisted together with 0.5 turn per inch to give a yarn of 210 grams tenacity was cut into predetermined lengths which were dipped in a solution of 15% by weight of diacetin (glycerol diacetate) in water. The wet lengths of yarn were squeezed to a liquid pick-up of about 60% by weight. Parallel yarns were laid longitudinally on the web with  $\frac{1}{8}$

inch spaces therebetween. Yarns were also laid transversely at  $\frac{1}{8}$  inch intervals, resting on the longitudinal yarns. Another web identical with the first was placed on the stack, heavy paper was placed on top and a hot iron was passed over the assembly several times to produce a composite structure as shown in FIG. 2. This can be used as the outer cover for sanitary napkins.

#### Example II

The procedure of Example I can be repeated, substituting for the high tenacity rayon yarns 50 denier nylon yarns alternated with 50 denier cellulose acetate yarns, the warp-wise yarns being spaced 8 to the inch and the transverse yarns being spaced 4 to the inch. The resulting non-woven product can be employed as the outer cover for a sanitary napkin constructed as shown in FIG. 3.

It is to be understood that the foregoing detailed description is given merely by way of illustration and that many variations may be made therein without departing from the spirit of our invention.

Having described our invention what we desire to secure by Letters Patent is:

1. A strong, flexible, non-woven, fibrous, laminate structure comprising at least one non-woven fibrous plasticizable web and a plurality of reinforcing yarns in substantially the same plane, on at least one surface of said web, said yarns carrying a plasticizer for the fibers of said web, said web fibers being plasticized to render them adherent to said yarns only at the points of contact with said yarns and said yarns being bonded to said web only by said plasticized fibers.

2. A non-woven structure according to claim 1, wherein in some of said yarns extend in one direction and others of said yarns overlie said first-named yarns and extend in a second direction to afford reinforcement in a plurality of directions, migration of said plasticizer bonding said yarns to each other as well as to said web.

3. A non-woven structure according to claim 1, wherein in at least some of said yarns have a tenacity of at least about 3.0 grams per denier, the denier of the yarns varying from about 30 to about 150.

4. A non-woven structure according to claim 1, wherein in at least some of said yarns comprise fibers to which said activating agent is inert.

5. A non-woven structure according to claim 1, wherein in said yarns comprise rayon produced by saponification of cellulose acetate and having a tenacity of at least about 5.0 grams per denier.

6. A non-woven structure according to claim 1, wherein in said yarns comprise nylon.

7. A non-woven structure according to claim 1, wherein in said non-woven web comprises cellulose acetate fibers.

8. A non-woven structure according to claim 1 including a second non-woven fibrous plasticizable web disposed on the other surface of the plane in which said yarns lie, said second web being bonded to said first web and to said yarns by the action of said plasticizer.

9. A non-woven structure according to claim 1, wherein in said plasticizer is a liquid of low volatility.

10. A sanitary napkin comprising in combination a covering as claimed in claim 1 and an adsorptive, non-woven fibrous pad contained within said covering.

11. A sanitary napkin according to claim 10, wherein said covering includes a second non-woven fibrous plasticizable web disposed on the other surface of the plane in which said yarns lie, said second web being bonded to said first web and to said yarns by the action of said plasticizer.

12. A sanitary napkin according to claim 10, wherein said non-woven webs comprise cellulose acetate.

13. A sanitary napkin according to claim 10, wherein said yarns comprise rayon produced by saponification of cellulose acetate and having a tenacity of at least about 5.0 grams per denier.

14. A sanitary napkin according to claim 10, wherein said high-tenacity yarns comprise nylon.

15. A sanitary napkin according to claim 10, wherein said plasticizer is a liquid of low volatility.

16. The method of forming a strong fibrous structure which comprises forming a fibrous structure of potentially adhesive fibers positioning a multiplicity of substantially uniplanar yarns containing an activating agent for said potentially adhesive fibers adjacent said fibers, and bonding said yarns to said potentially adhesive fibers through the action of said activating agent.

17. The method according to claim 16, wherein said potentially adhesive fibers are present in a non-woven web and said inert fibers are present in a yarn serving as a reinforcement for said non-woven web.

18. The method according to claim 16 wherein said inert fibers comprise rayon produced by saponification of cellulose acetate and having a tenacity of at least about 5.0 grams per denier.

19. The method according to claim 16 wherein said potentially adhesive fibers comprise cellulose acetate.

20. The method according to claim 16, wherein said potentially adhesive fibers are plasticizable and said activating agent comprises a liquid plasticizer for said potentially adhesive fibers, said liquid plasticizer being of low volatility.

21. A method of preparing a laminated, reinforced, non-woven, fibrous, soft sheet structure having high strength comprising placing a non-woven web which in-

cludes potentially adhesive fibers on a support, superposing on said web in substantially the same plane a plurality of yarns containing an activating agent for said potentially adhesive fibers, and applying heat and pressure to said web and yarns whereby said activating agent causes said potentially adhesive fibers to adhere to one another and to said yarns.

22. A method of preparing a non-woven structure according to claim 21, wherein some of said yarns extend in one direction and others are placed to overlie said first-named yarns and extend in a second direction to afford reinforcement in a plurality of directions, application of heat and pressure bonding said yarns to one another at their cross-over points.

23. A method of preparing a non-woven structure according to claim 21 including the step of positioning a second non-woven web over said yarns prior to applying heat and pressure, said second non-woven web including potentially adhesive fibers also attacked by said activating agent, whereby said second web is bonded to said first-named web as well as to said yarns.

**References Cited in the file of this patent**

**UNITED STATES PATENTS**

|           |                       |               |
|-----------|-----------------------|---------------|
| 2,294,898 | Fourness et al. ----- | Sept. 8, 1942 |
| 2,705,498 | Johnson -----         | Apr. 5, 1955  |
| 2,833,283 | Spahr et al. -----    | May 6, 1958   |
| 2,900,980 | Harwood -----         | Aug. 25, 1959 |